

# UNITED STATES PATENT OFFICE.

PETER SCHMID, OF BASEL, SWITZERLAND.

## PROCESS FOR PRODUCING WEIGHTED PILE-YARN FOR COLORED VELVETS.

1,102,088.

Specification of Letters Patent. Patented June 30, 1914.

No Drawing.

Application filed December 12, 1911. Serial No. 665,272.

*To all whom it may concern:*

Be it known that I, PETER SCHMID, merchant, a citizen of the Swiss Republic, and resident of Basel, Switzerland, have invented a new and useful Process for Producing Weighted Pile-Yarn for Colored Velvets.

My invention relates to an improved process for producing weighted pile yarn for colored velvets, and it consists in the steps 10 and processes herein described and claimed.

The object of my invention is to provide an improved weighted pile yarn for colored velvets, in which the silk fibers retain their original structure and qualities and are uniformly ungummed to permit a regular and uniform penetration of tin salts and similar weighting substances; thereby preventing an irregular and lumpy deposition of the weighting substances, and enabling 20 the pile to be evenly cut to provide a smooth and lustrous velvet.

Numerous efforts have been made to produce a chappe-yarn retaining the original structure of the silk fibers and uniformly 25 ungummed, to permit an even and uniform penetration of tin salts and similar weighting substances, in order to furnish weighted pile yarn for weaving colored velvets, which could be evenly cut to furnish a lustrous 30 velvet. It has been generally recognized in the trade that such use of chappe-yarn would be of great value in producing cheaper colored velvets, such as is done at present in the manufacture of black velvet, 35 which is weighted with vegetable substances instead of mineral salts.

Heretofore, the chappe-yarn formed from silk wastes have been ungummed by treating either the silk wastes or the yarns in various 40 different manners, but none of the previous processes have produced a uniformly ungummed chappe-yarn capable of use as weighted pile yarn in weaving colored velvets. In a Patent #848605, granted to me 45 on March 26, 1907, a process is disclosed for ungumming silk wastes, yarns, and tissues by treating them with soap lather, and said patent states that the treatment can be repeated a second time for removing a further 50 portion of the gum. The process disclosed

in this prior patent is for treating the silk in only one state or form, such as either wastes, yarns, or tissues, and said process does not insure the uniform ungumming of the silk with a retention of the original 55 structure of the fibers necessary for an even and uniform penetration of the weighting metallic salts.

By my improved process, the silk wastes are treated with soap lather for removing 60 a portion of the gum without injuring the original structure of the fibers. The fibers are then combed and spun into yarn, which is treated with soap lather to remove the final portion of the gum, and the fibers are 65 then weighted and dyed. This novel process of treating the silk with soap lather successively in the form of wastes and yarns produces an absolutely uniform ungumming and preserves the original structure of the 70 fibers; thereby providing a yarn which will be regularly and uniformly penetrated by weighting metallic salts. In this production of pile yarn, I preferably employ weighting substances equal to from 40% to 60% of the 75 silk:

My invention renders possible the advantageous manufacture of weighted colored velvets, and also permits the use of lower quality of silk wastes in the production of pile yarn. 80

I claim:—

The herein described process for producing weighted pile yarn for colored velvets, which consists in treating silk wastes with 85 soap lather for ungumming the latter without injuring the original structure of the silk fibers, then combing and spinning the silk wastes to form yarn, then treating the 90 yarn with soap lather to produce a regular and uniform ungumming thereof, and then weighting and dyeing the yarn.

In witness whereof I have hereunto signed my name this 29th day of November, 1911, in the presence of two subscribing witnesses. 95

PETER SCHMID.

Witnesses:

GEO. GIFFORD,  
AMAND RITTER.